

Feb. 25, 1969

J. E. MEE

3,429,740

GROWING GARNET ON NON-GARNET SINGLE CRYSTAL

Filed Sept. 24, 1965



INVENTOR

JACK E. MEE

BY

*Robert G. Rogers*

ATTORNEY

1

3,429,740

GROWING GARNET ON NON-GARNET  
SINGLE CRYSTAL

Jack E. Mee, Anaheim, Calif., assignor to  
North American Rockwell Corporation  
Filed Sept. 24, 1965, Ser. No. 489,930

U.S. Cl. 117—106  
Int. Cl. B01j 17/30

9 Claims

ABSTRACT OF THE DISCLOSURE

An article comprising a monocrystalline substrate of non-garnet material, and a film of monocrystalline garnet epitaxially disposed on the substrate. The composite may be prepared by vaporizing halides of the garnet constituent metals, and transporting the resultant halide vapors substrate and an oxygen-providing gas to adjacent the heated substrate, thereby causing a garnet to deposit epitaxially on the substrate.

This invention relates to garnet crystals grown on non-garnet substrates and to a chemical vapor deposition process for growing garnet crystals epitaxially on non-garnet substrates.

Crystals with the garnet structure have become important technologically and scientifically in recent years. Many of the crystals have magnetic properties which make them useful for device purposes. For example, thin crystals of certain of the magnetic garnets are transparent and display a magneto-optic effect when polarized light impinges on the crystal. Such magneto-optic effect can be used for display purposes. Scientifically, this effect can be used to study magnetic domain structures, electronic absorption spectra, etc. Even non-magnetic garnets have useful device properties, e.g.,  $Y_3Al_5O_{12}$  may be used as a laser host material.

Single crystal garnets are grown by Verneuil, hydrothermal and flux techniques. Commercially they are usually grown by the flux techniques wherein the garnet is grown from a molten salt solution. These methods are not adaptable to growing high quality, thin single crystal garnet films.

It is important to have the films as free of defects as possible in order to make the greatest use of them. This is best accomplished by chemical vapor deposition since the garnet films can be used as grown whereas garnets grown by other techniques must be cut and mechanically polished thereby introducing many defects.

The characterizing feature of this invention is a composite of single crystal garnet on a single crystal substrate which is not within the garnet class. The epitaxial single crystal garnet film may be grown by a chemical vapor deposition process on large areas.

Garnet is defined herein as a solid material having the formula  $\{M_3'\}[M_2'''](M_3''')O_{12}$  where  $M'$  is defined herein as at least one element selected from the class consisting of Y, La, Pr, Nd, Sm, Eu, Gd, Tb, Dy, Ho, Er, Ym, Yb, Lu, Ca and Bi;  $M''$  is defined herein as at least one element selected from the class consisting of Fe, In, Sc, Mg, Zr, Sb, Al and Ga; and  $M'''$  is defined herein as at least one element selected from the class consisting of Fe, Al, Ga, Si, Ge and V. Particularly preferred because of their magnetic properties are the rare earth iron garnets. Particularly preferred of this class of garnet materials are  $Y_3Fe_5O_{12}$  and  $Gd_3Fe_5O_{12}$ , while the preferred non-magnetic garnet is  $Y_3Al_5O_{12}$ .

In the above formula, the notations  $\{ \}$ ,  $[ \ ]$ ,  $( \ )$ , represent sites in the garnet material designated  $c$ ,  $a$ , and  $d$  sites respectively. Elements known to exist in these sites in the garnets are listed below and designated as to their oxidation state:

2

$c$  sites— $Y^{3+}$ ,  $La^{3+}$ ,  $Pr^{3+}$ ,  $Nd^{3+}$ ,  $Sm^{3+}$ ,  $Eu^{3+}$ ,  $Gd^{3+}$ ,  $Tb^{3+}$ ,  $Dy^{3+}$ ,  $Ho^{3+}$ ,  $Er^{3+}$ ,  $Tm^{3+}$ ,  $Yb^{3+}$ ,  $Lu^{3+}$ ,  $Ca^{2+}$ ,  $Bi^{3+}$ .  
 $a$  sites— $Fe^{3+}$ ,  $In^{3+}$ ,  $Sc^{3+}$ ,  $Mg^{2+}$ ,  $Zr^{4+}$ ,  $Sb^{5+}$ ,  $Al^{3+}$ ,  $Ga^{3+}$ .  
 $d$  sites— $Fe^{3+}$ ,  $Al^{3+}$ ,  $Ga^{3+}$ ,  $Si^{4+}$ ,  $Ge^{4+}$ ,  $V^{5+}$ .

5 Garnets may be defined as pure, mixed or substituted. Typical examples of pure garnets are  $Y_3Fe_5O_{12}$ , and  $Tb_3Fe_5O_{12}$ . Examples of mixed garnets include

$La_xY_{3-x}Fe_5O_{12}$

10  $Pr_xY_{3-x}Fe_5O_{12}$ ,  $Nd_xY_{3-x}Fe_5O_{12}$ ,  $Nd_xGd_{3-x}Fe_5O_{12}$ ,  
 $Nd_xSm_{3-x}Fe_5O_{12}$

where  $x$  may have a maximum value of 0.5, 1.3, 2, 1.4, 0.35 respectively for the preceding examples. Although La,

15 Pr and Nd exist in mixed garnets, they do not exist in pure garnets such as  $La_3Fe_5O_{12}$ ,  $Pr_3Fe_5O_{12}$ , and  $Nd_3Fe_5O_{12}$ . A garnet with any other type of substitution is called a substitution garnet, for example,  $\{Y_3\}[Fe_2](Fe_{3-x}Al_x)O_{12}$ , and  $\{Gd_{3-x}Ca_x\}[Fe_2](Fe_{3-x}Si_x)O_{12}$ .

20 Other Fe containing garnets include  $Sm_3Fe_5O_{12}$ ,

$Eu_3Fe_5O_{12}$

$Dy_3Fe_5O_{12}$ ,  $Gd_3Fe_5O_{12}$ ,  $Ho_3Fe_5O_{12}$ ,  $Er_3Fe_5O_{12}$ ,  $Tm_3Fe_5O_{12}$ ,  
25  $Yb_3Fe_5O_{12}$ ,  $Lu_3Fe_5O_{12}$ . The classical garnet is

$Ca_3Fe_2Si_3O_{12}$

It is an object of this invention to provide single crystal garnet crystallographically bonded to a single crystal non-garnet structure.

30 Another object of this invention is to provide a composition having a large area of single crystal garnet on a non-garnet substrate.

Still another object of this invention is to provide a process for producing single crystal garnet on single crystal non-garnet substrates in large quantities.

These and other objects of this invention will become more apparent when considered in connection with the following description and drawings in which:

FIGURE 1 is a representation of an apparatus used 40 in growing single crystal garnet on a single crystal non-garnet substrate.

Referring now to FIGURE 1, the apparatus of the present invention comprises a chamber 1, including inlet means 2 for injecting gases into one end of the chamber 45 1, and an exhaust 5 at the other end of the chamber. The chamber is surrounded by heater elements 6, 7 and 8 for controlling the temperature at locations within the chamber. Supported inside chamber 1 are a plurality of spaced crucibles 10 and 11. The crucibles are spaced to be within

50 the area heated by respective heater elements. Also within the chamber is a quartz holder 13 on which substrates or seed crystals 12 are supported. The terms substrate and crystals are used interchangeably herein. The crystals are located in chamber 1 so that they are exposed to a mixture of gases flowing from inlets 2 and 14. Inlet 2 is connected to a source (not shown) of inert carrier gases such as helium and argon. Inlet 14 is connected to a source (not shown) of gases such as oxygen and water vapor, carbon dioxide and hydrogen.

55 The substrates 12 on which the garnet crystal material is deposited or grown are comprised of single crystal non-garnet type materials. For purposes of describing the composition produced by the process, the substrate material selected is  $MgO$ , although other substrate materials, for example,  $MgAl_2O_4$ ,  $\alpha$ - $Al_2O_3$ , and other materials having the formula  $Me'Me_2''O_4$  may also be utilized in producing the structure. The term  $Me'$  may be Li, Mg, Mn, Fe, Co, Ni, Cu, Zn, or Cd and  $Me''$  may be Al, Cr, Mn, Fe, Ti.

60 It should be pointed out that the process is not limited to the particular chamber illustrated in FIGURE 1. Other chambers such as that described in an application entitled  
70

"Ferrite Memory Device," Ser. No. 428,158, filed Jan. 26, 1965 may also be used as well as the chambers described in an application entitled "Epitaxial Dielectric MgO Crystals," Ser. No. 424,417, filed Jan. 8, 1965, now U.S. Patent No. 3,386,852. The chamber components may be comprised of quartz, alumina or other suitable materials not causing contamination of the resulting garnet structure.

The substrates **12** may be prepared by cleaving optical grade MgO along a {100} cleavage plane or by cutting the MgO in the plane of desired configuration along its other crystal faces. The substrates are ground flat to produce a crystal having a selected size and a selected crystallographic plane and chemically polished in an acid etch solution. The substrates **12** are supported on the holder **13** inside chamber **1** and a garnet layer may be deposited as described in detail hereinafter.

The source materials **15** and **16** for producing the garnet deposit on the substrates **12** are placed in containers **10** and **11** and heated to vaporization by heater elements **6** and **7** respectively. Metal halides used as source materials are placed inside containers **10** and **11**. The halides include those of the metallic elements Y, La, Pr, Nd, Sm, Eu, Gd, Tb, Dy, Ho, Er, Tm, Yb, Lu, Ca and Bi in one container, and Fe, In, Sc, Mg, Zr, Sb, Al, Ga, Si, Ge and V in the other. When heated, the solid metal halides slowly vaporize.

Simultaneously with the heating of the above materials **15** and **16**, the above described gases are emitted through inlets **2** and **14**. The plurality of gases including a source of available oxygen and the source material vapors react at the heated surface of the substrate to epitaxially deposit single crystal garnet on the non-garnet substrates.

After the garnet layer has been deposited on the substrate, the composition may be removed and placed in other environments, for example, a conventional vacuum deposition chamber (not shown) for further processing, depending upon the particular use intended for the composition.

To form the preferred rare-earth iron garnet structures, the corresponding halides of iron and of the desired rare earth metals are selected. Thus to form the particularly preferred structures the halides of yttrium, gadolinium and iron will be utilized. The choice of particular halide, such as chloride, bromide, iodide or fluoride will be determined by its decomposition temperature and other factors known to those skilled in the art.

The practice of the inventive methods for producing a single crystal garnet crystal on a non-garnet crystal substrate is described more fully with reference to the following examples:

#### Example I

A substrate material, MgO, is prepared by cleaving the crystal along a {100} cleavage plane into approximately 18 mm. x 12 mm. dimensions. After cleaving, the substrate is mechanically ground flat on a series of metallographic papers to the 4/0 size. They are then chemically polished in a concentrated H<sub>3</sub>PO<sub>4</sub> etching solution heated to 125° C. for 20 minutes. After the etching the substrates are given a thorough hot water rinse.

A quartz or alumina cylindrical shaped apparatus of FIGURE 1 having a 54 mm. I.D. is utilized as the deposition chamber. A quartz or alumina holder is used to support the MgO crystal in the middle of the chamber. Quartz or alumina crucibles **10** and **11** contain source materials **15** and **16**. The crucibles are each carefully located in the chamber with each source material having individually controlled electrical heater elements **6** and **7**. In this example, the source materials are the metal halides FeBr<sub>2</sub> and YCl<sub>3</sub>. The temperature for the FeBr<sub>2</sub> is held at 700° C. and the YCl<sub>3</sub> is held at 1150° C. to give sufficient vapor pressures for the two reactants. The crystal is maintained at 1150° C. After the crystals and the containers are properly located in the chamber and heated to the appropriate temperature, argon at 1 ft.<sup>3</sup>/hr. is passed through inlet **2** and carries the FeBr<sub>2</sub> and YCl<sub>3</sub>

vapors to the MgO crystal. Oxygen at 1 ft.<sup>3</sup>/hr. is bubbled through water at room temperature and brought into the reaction area just in front of the MgO crystal through the opening provided by a 10 mm. I.D. Vycor or alumina tube at one end of the chamber, shown in FIGURE 1 as opening **14**. The H<sub>2</sub>O, O<sub>2</sub>, FeBr<sub>2</sub>, and YCl<sub>3</sub> vapors react in the area of the MgO crystal. The reaction is continued for one hour, then the furnaces and the substrate are permitted to cool for approximately two hours. The garnet film formed is approximately five microns thick over an area of 18 mm. x 12 mm. The film displays the characteristics ferromagnetic properties of yttrium iron garnet and is identified by X-ray diffraction techniques.

The reaction to form the garnet layer can be represented as follows:



where <sub>(g)</sub> is gas and <sub>(s)</sub> is solid.

#### Example II

The process and apparatus as described in connection with Example I is utilized in this example except that AlCl<sub>3</sub> at 180° C. and YCl<sub>3</sub> at 1150° C. are used in place of the source materials described therein. Instead of oxygen, argon is bubbled through water to produce an H<sub>2</sub>O vapor. The reaction to form the garnet layer can be represented as follows:



#### Example III

The process and apparatus as described in connection with Example I is utilized in this example except that in lieu of the MgO crystal prepared as described, a flat  $\alpha$ -Al<sub>2</sub>O<sub>3</sub> (sapphire) crystal which has been mechanically and chemically polished is used as the substrate. GdCl<sub>3</sub> is used in place of YCl<sub>3</sub>. The reaction to form the garnet layer can be represented as follows:



#### Example IV

The process and apparatus as described in connection with Example I is utilized in this example, except that GdI<sub>3</sub> at ~1000° C. is used in place of the YCl<sub>3</sub>. The reaction to form the garnet layer can be represented as follows:



#### Example V

The process and apparatus as described in connection with Example I is utilized except that a {110} MgO plane is used as the substrate rather than a {100} cleavage plane. The {110} plane is prepared by properly orienting the MgO crystal, cutting it with a diamond saw, determining the orientation by X-ray Laue techniques, mechanically polishing and then chemically polishing. The chemical polishing is done by soaking the crystals in a 3:1 H<sub>3</sub>PO<sub>4</sub>: H<sub>2</sub>SO<sub>4</sub> solution at 100–120° C. followed by a hot water rinse, a dilute 10% HCl rinse, and a final distilled water rinse.

## Example VI

The process and apparatus as described in Example V except that a {111} MgO plane is used rather than a {110} plane.

## Example VII

The process and apparatus as described in Example I except that a {110} or {111} MgO plane is used rather than a {100} plane and  $\text{GdBr}_3$  is used rather than  $\text{YCl}_3$ . The reaction to form the garnet layer can be represented 10 as follows:



I claim:

1. A composite comprising a monocrystalline substrate of non-garnet material and an epitaxial film of single crystal garnet material on said substrate, said substrate being selected from the class consisting of  $\text{MgO}$ ,  $\alpha\text{-Al}_2\text{O}_3$  and  $\text{Me}'\text{Me}''_2\text{O}_4$  wherein  $\text{Me}'$  is selected from the class consisting of Li, Mg, Mn, Fe, Co, Ni, Cu, Zn and Cd and wherein  $\text{Me}''$  is selected from the class consisting of Al, Cr, Mn, Fe and Ti.

2. A composite according to claim 1 wherein said single crystal garnet material is selected from the class consisting of  $\text{Y}_3\text{Fe}_5\text{O}_{12}$ ,  $\text{Gd}_3\text{Fe}_5\text{O}_{12}$  and  $\text{Y}_3\text{Al}_5\text{O}_{12}$ .

3. A composite according to claim 1 wherein said single crystal garnet material is  $\text{Y}_3\text{Fe}_5\text{O}_{12}$  and wherein said substrate is single crystal  $\text{MgO}$ .

4. A process for epitaxially growing garnet single crystals on a non-garnet single crystal substrate selected from the class consisting of  $\text{MgO}$ ,  $\alpha\text{-Al}_2\text{O}_3$  and  $\text{Me}'\text{Me}''_2\text{O}_4$  wherein  $\text{Me}'$  is selected from the class consisting of Li, Mg, Mn, Fe, Co, Ni, Cu, Zn, and Cd and

wherein  $\text{Me}''$  is selected from the class consisting of Al, Cr, Mn, Fe and Ti, said process comprising the steps of: heating said substrate, vaporizing halides of the constituent metals of said garnet, and transporting said vaporizing halides and an oxygen-providing gas to adjacent said heated substrate, whereby said halides and said gas react at said heated non-garnet substrate to deposit epitaxially a single crystal garnet film on said substrate.

5. The process as recited in claim 4 wherein said gases include decomposable halides of iron and of the rare-earth metals.

6. The process as recited in claim 4 wherein said substrate comprises  $\text{MgO}$  having a {100} deposition surface, and wherein said halides include an iron halide and at least one rare-earth metal halide selected from the class consisting of gadolinium and yttrium halides.

7. The process as recited in claim 4 wherein said deposited garnet crystal film is selected from the class consisting of  $\text{Y}_3\text{Fe}_5\text{O}_{12}$ ,  $\text{Gd}_3\text{Fe}_5\text{O}_{12}$  and  $\text{Y}_3\text{Al}_5\text{O}_{12}$ .

8. The process as recited in claim 4 wherein said halides include a yttrium halide and an aluminum halide.

25 9. The process as recited in claim 4 wherein said vaporized halides are transported in an inert carrier gas.

## References Cited

## UNITED STATES PATENTS

3,131,082 4/1964 Gambino ----- 117—106 X

ALFRED L. LEAVITT, Primary Examiner.

A. GOLIAN, Assistant Examiner.

U.S. Cl. X.R.

117—169, 234, 235; 106—42